

Patented Feb. 15, 1927.

1,617,996

# UNITED STATES PATENT OFFICE.

CARLETON ELLIS, OF MONTCLAIR, NEW JERSEY, ASSIGNOR TO CHADELOID CHEMICAL COMPANY, OF NEW YORK, N. Y., A CORPORATION OF WEST VIRGINIA.

## FLAME-COLORING AGENT.

No Drawing.

Application filed December 22, 1925. Serial No. 77,122.

This invention relates to a composition of matter adapted to produce in the flames of an ordinary hearth-fire in which a wood is a combustible, one or more colors of a vivid 5 character more or less resembling the colors of a driftwood blaze.

Powders containing salts giving different colors have been used but they exhibit the disadvantage that often particles are carried away in the draft and the coarser and heavier particles are likely to fall through the crevices of a wood fire and become buried in the ashes and therefore ineffective. Usually the coloration produced by such powders is of relatively short duration, lasting 15 not more than a few minutes.

In the present invention flame-coloring compounds or substances are employed which are cemented together in some suitable manner, as for example by means of a 20 binder preferably of a fusible combustible character.

A flame-coloring agent is used which freely tinges or tones the flame under the 25 temperature conditions of an ordinary open-fire or hearth-fire burning wood.

This therefore usually excludes such substances as boric acid or copper carbonate and the like from the preferred embodiment 30 of the invention. Chlorides of certain metals are best adapted for the purpose, cuprous or cupric chloride being satisfactory to obtain certain tones. The latter compounds give a violet to a green color of a pleasant character and at relatively low flame temperatures. Strontium chloride may be used to obtain a crimson coloration, barium chloride for green, and so forth.

The binder as stated is fusible and combustible preferably carbonizing or intumescent to yield a mass from which the coloring agent is relatively slowly liberated. Rosin, wax, gilsonite, pitch and the like are preferred as these substances may serve to 45 seal the chemical compounds, many of which are hygroscopic and thereby prevent any unsightly discoloration of the packages in which the product is shipped, furthermore conferring keeping qualities in some cases 50 on some salts which are of an unstable character.

The amount of the binding agent may be varied for example it may be just sufficient to bind together the powder or granular 55 flame-coloring chemical materials but pref-

erably an amount of binder is employed sufficient to allow melting or casting to definite shapes, e. g. sheets, cubes, tablets, discs, wafers and the like. Sometimes the binding agent may have inherent flame-coloring 60 properties as for example tetrachlornaphthalene, copper stearate, and so forth, are employed.

By embedding the flame-coloring salts or compounds in the combustible sealing agent 65 excellent keeping qualities are conferred on substances which otherwise might be affected by protracted exposure in ordinary paper or paste-board shipping packages. Of the binders, etc. above stated, wax (e. g. ordinary 70 paraffin wax, as herein mentioned) gilsonite, etc., give very water resistant products, which will keep well, in cardboard or paper packages, any hygroscopic properties of the salts present being effectively counteracted 75 by the sealing vehicle. Rosin exercises such an effect also, to a certain degree.

In using the product of the present invention one or more fragments, tablets, discs and the like are placed on the top of the mass of wood or elsewhere in the structure assembled on the hearth. This may be done at the time the fire is built. When the fire is started these tablets or in whatever shape the product of the present invention is employed will be found to fuse or become sticky and therefore do not drop through the crevices of the wood structure to the bottom but remain in the upper part of the fire where contact of the flames will produce the maximum coloring effect. By remaining thus adherent to the burning wood in this effective position the flames become very quickly tinged with vivid colors.

When the organic binder carbonizes it 80 appears to seal some of the flame-coloring agent in some manner so that it is more gradually liberated as combustion progresses. This feature of more lasting flame-coloration is a desirable one.

The tablets or masses of the composition may be added from time to time as the fire progresses or as new fuel is introduced.

One composition which I have found suitable for the purpose is made by melting ordinary rosin and adding thereto an equal weight of cupric chloride (ordinary crystallized compound) previously ground to a course powder. After stirring to mix the ingredients sufficiently the composition is 105 110

100  
poured on to a flat surface and subsequently broken into fragments say one-fourth to one-half inch in diameter. Usually I prefer to pour the composition at such a temperature that it is obtained as a thin sheet not more than one-eighth to one-fourth of an inch in thickness. Another composition is made by taking forty-five parts by weight of cupric chloride, grinding with four parts lamp black and adding to twenty-two parts of molten paraffin wax. A black composition is obtained which I find may be poured on a glass or enamel surface to make discs or flat pieces, from one-half to one inch in diameter, which are excellent in their adherence to wood as soon as slightly softened by heat. The term "disc" or the term "diameter" is not intended to exclude all shapes other than circular and obviously by breaking up the sheets, pieces of more or less irregular shape may be produced. The salts of copper, barium, strontium, etc., mentioned above, which give distinctive or pronounced coloration to the flames may be embraced in the expression "flame coloring salt of an earth metal." The paraffin wax may contain ten to twenty per cent of a hard wax such as carnauba in order to obtain a product which in warm weather in the package does not coalesce. Strontium chloride as noted above may be substituted for the copper chloride. In this way a package can be prepared containing tablets or fragments of substantial size each of which has a characteristic flame-coloring agent and on distributing several of these in the fire different colors are produced in different parts of the hearth.

105  
In addition to the binders mentioned above others which have not the same waterproofing effect but which have good binding power, such for example as casein or glue, and in some cases dextrine, starch and the like may be used but are not recommended in preparing the preferred form of the present invention.

110  
Preferably no oxygen yielding substances such as nitre, potassium chlorate, and so forth, are present as thereby pyrotechnical effects not desired in the present case would result. At any event I do not use such amounts of highly oxidizing substances as would produce anything such as would constitute pyrotechnic compositions, fuzees, Fourth of July fire works, or the like. It is an object of the present invention to obtain the slow liberation of the flame-coloring agent, so that a few tablets might last for an entire evening.

115  
60 The combustible binder may be extended and rendered less combustible in some cases by using inert bodies, e. g. clay or other earthy material. Infusorial earth which is quite porous may be impregnated with aqueous solutions of the salts employed for

120  
flame-coloration, the earth dried and then this material embedded in resin, wax, pitch or other binder. The object in this case is to secure a greater retardation of the liberation of the flame-coloring agent.

70  
In some cases it is possible to employ a mineral binder with the flame-coloring agent, e. g. magnesium oxide chloride cement to contain the copper or other flame-coloring salts.

75  
I have observed, however, that a product of this kind is relatively heavy and does not adhere to wood hence when the fuel settles or is disturbed these mineral tablets very easily fall through the fire structure and their flame-coloring effect is then practically lost. It appears to be necessary to secure the maximum effect to have the flame-coloring agent remain above the lower part of the fire bed and this result is achieved by employing the fusible binder or one which softens by heat sufficiently to readily adhere to wood.

80  
85  
In some cases mixtures of various binders, such as rosin, gilsonite and the like, may be mixed together to prepare a binder having a particular softening point.

90  
95  
Again when pouring the composition on a flat surface it is possible to make a pouring first with a composition giving a certain color, e. g. blue, applying to the surface irregularly so as to make bands or local deposits and immediately fill in around these with a second composition, e. g. barium chloride, so that a coloring agent is obtained 100 with striations or bands of the composition containing different coloring agents. On breaking these into fragments many of them were found to give a two-tone or three-tone flame-coloration as the case may be. While 105 as stated I prefer to cast or mold the composition to any suitable shape it is also possible to apply in the molten state to a chill-roll to make a flakelike product.

110  
Although I prefer tablets or discs or pieces about one-eighth inch thick and one-half inch to one inch in diameter the size may be varied or an assortment of sizes may be used in each package.

115  
Various pigments may be added, e. g. red, ochre or amber, lamp black, and so forth, to give the fragments or tablets a characteristic appearance by means of which a tablet giving any particular flame-color may be recognized.

120  
125  
The term "tablet" is intended to cover or embrace a mass of the composition of the present invention of any appropriate shape including irregular fragments or flakes of a size appropriate to apply to a fire of the character described. Two large masses in the fire at one spot give so extensive a coloration that they would not thereby appropriately simulate the effect of driftwood. On the other hand particles which are very

small are ineffective and transient in their coloring effect. Hence I prefer not to employ the composition in the form of a fine powder.

5 It will be noted that the binders which I have above mentioned as the preferred examples thereof, are not soluble in water, are capable of at least partially melting at temperatures substantially above that of the 10 human body (98° F. or so) but which do not substantially melt at below body temperature, the said substances being generally "oil-soluble", organic substances. Such substances are hereinafter referred to as "relatively 15 high melting, water-insoluble oil-soluble organic binders".

What I claim is:

1. A substantially waterproofed composition of matter adapted to cause hearth burning wood to produce flames of variegated colors, comprising a flame-coloring agent embedded in a fusible combustible binder made up into pieces of such size as to produce effective flame coloration lasting for 25 substantially more than a few seconds, when placed on such fire.

2. Substantially waterproofed tablets capable of being placed on a burning wood fire without explosion comprising a flame-coloring metallic chloride held in a fusible combustible binder made up into pieces of such size as to produce effective flame coloration lasting for substantially more than a few seconds, when placed on such fire.

3. A composition of matter adapted to cause hearth-fires burning wood to produce variegated colors, which comprises a flame-coloring agent embedded in a combustible fusible binder, substantially free from compounds of an oxidizing nature; said flame-coloring agent being adapted to readily tinge flame at the temperature of burning wood.

4. A composition of matter comprising cupric chloride embedded in a waxy waterproofing binder.

5. A composition of matter comprising cupric chloride in copper stearate.

6. A hearth-fire flame-coloring composition in tablet form containing a water-insoluble somewhat fusible binder, the tablets

being of such size and composition as to produce effective flame coloration lasting for substantially more than a few seconds, when placed on a wood fire.

7. A hearth-fire flame-coloring composition in tablet form adapted at an elevated temperature substantially below that of the flame of a wood fire, to adhere to wood made up into pieces of such size as to produce effective flame coloration lasting for substantially more than a few seconds, when placed on a wood fire. 55

8. A tablet containing a flame coloring salt of an earth metal and a somewhat fusible binder, capable of at least partially melting at a temperature substantially above normal human body temperature but not melting at normal human body temperature. 60

9. A non-explosive tablet containing a flame coloring salt of an earth metal and a relatively high melting water-insoluble oil-soluble organic binder, said tablet being of sufficient size to give an effective flame coloration lasting for substantially longer than a few seconds. 65

10. A non-explosive tablet containing a flame coloring chloride of an earth metal and a relatively high melting water-insoluble oil-soluble organic binder, said tablet being of sufficient size to give an effective flame coloration lasting for substantially longer than a few seconds. 70

11. A non-explosive tablet containing a flame coloring salt of an earth metal and a relatively high melting water-insoluble oil-soluble organic binder, such binder including paraffin wax, said tablet being of sufficient size to give an effective flame coloration lasting for substantially longer than a few seconds. 75

12. A non-explosive tablet containing a flame coloring salt of an earth metal and a relatively high melting water-insoluble oil-soluble organic binder, such binder including paraffin wax and an agent capable of raising the melting point thereof, said tablet being of sufficient size to give an effective flame coloration lasting for substantially longer than a few seconds. 80

CARLETON ELLIS.